

# UNITED STATES PATENT OFFICE.

FRANÇOIS BOREL, OF CORTAILLOD, SWITZERLAND, ASSIGNOR TO THE SOCIÉTÉ ANONYME DE CÂBLES ÉLECTRIQUES, (SYSTÈME BERTHOUD, BOREL & CIE.,) OF PARIS, FRANCE.

## INSULATING MATERIAL FOR ELECTRICAL CONDUCTORS.

SPECIFICATION forming part of Letters Patent No. 258,549, dated May 30, 1882.

Application filed April 15, 1882. (No specimens.) Patented in France March 4, 1882, in Germany March 15, 1882, and in England March 29, 1882.

*To all whom it may concern:*

Be it known that I, FRANÇOIS BOREL, of Cortaillod, Switzerland, have invented a certain new and useful Improvement in Insulating Materials for Electrical Conductors, of which the following specification is a full description.

The present invention has reference more particularly to the manufacture of an electrical insulating material from a siccative oil—such as linseed-oil—by conversion into a solid elastic body.

The following is considered the best mode of carrying the invention into effect. In a suitable open vessel of metal linseed-oil is heated to the temperature of ebullition—say 320° centigrade. The heating-vessel not being covered, the oil is agitated all the time, so that the part in contact with the air is continually changing. The oil becomes blacker and blacker, so that at the end of, say, from twenty minutes to several hours, according to the quality of the oil, it is transformed into a solid elastic mass resembling caoutchouc. This material used alone as an insulating material is not perfectly satisfactory. It has been found that by mixing a resinous material—such as colophony (rosin)—with the oil when its transformation from a liquid to a solid begins a product is obtained which is insulating to the same degree as the mixture of colophony and paraffine, which has heretofore been employed by myself and others associated with me in the manufacture of cables. The quantity of colophony to be added to the oil depends upon the degree of hardness which it is desired to impart

to the material. With a weight of colophony equal to that of the oil a very elastic and highly insulating material is obtained, which is not hardened by cold. If the proportion of colophony is increased, the material becomes somewhat brittle.

As to the chemical action which takes place in the transformation of the liquid oil into a solid, it is probable that an oxidation in the presence of the air takes place, and also that there is a molecular change which it is impossible to determine.

The material prepared as described, with or without admixture of colophony, can be applied by methods and means heretofore employed as a coating directly upon the wire or conductor; or it can be used to impregnate fabric which may be wrapped around the conductor.

I claim—

1. As an insulating material or ingredient in insulating compounds, siccative oil—such as linseed-oil—transformed by heat into a solid body, substantially as described.

2. The combination, with siccative oil—such as linseed-oil—transformed into a solid by heat, of a resinous matter—such as colophony—substantially as described.

In witness whereof I have hereunto signed my name in the presence of two subscribing witnesses.

FRANÇOIS BOREL.

Witnesses:

ROBT. M. HOOPER,  
AMAND RITTER.